

# United States Patent Office

2,758,010

Patented Aug. 7, 1956

1

2,758,010

## METHOD OF CLAY TREATMENT

Ben W. Rowland, Hillside, N. J., assignor to Georgia Kaolin Company, Elizabeth, N. J., a corporation of New Jersey

No Drawing. Application June 10, 1949,  
Serial No. 98,410

9 Claims. (Cl. 23—110)

This invention relates to the treatment of clay and more particularly to a method of treating clay to improve its brightness. "Brightness," as herein used, is a relative term based upon the reflective power of a freshly prepared surface of magnesium oxide which is ordinarily taken as having 100% brightness.

Many of the commercial uses to which clay may be applied, e. g., clay for paper coating, demands a high degree of brightness. Because of the demand for brightness in clay for the paper industry, as well as for the ceramics and other clay consuming industries, many large deposits which might otherwise be accessible have not been developed.

It has been found that many clays which are suitable from the standpoint of physical characteristics other than brightness are so lacking in brightness as to be unsuitable for most commercial purposes.

Moreover, present methods of refinement, including present methods of bleaching, have not served to overcome this lack of brightness inherent in many clay deposits.

Brightness requirements must be considered in connection with color requirements. The practice of the orthodox bleaching processes may result in imparting a gray tone to the clay which renders it unsatisfactory. Clay in this condition is said to be "overbleached." It may be said that in general a clay on the buff side is more desirable than a clay on the gray side even if its brightness is somewhat lower. In consequence, the limit of brightness improvement in the treatment of clay, notably coating clay, has been the limit of brightness obtainable without changing such color as remains in the clay from buff to gray. It will be understood that although the amount of color difference present in coating clays generally is relatively small, it is usually observable by a side-to-side comparison of different specimens. In coating clays, a brightness difference of as much as three percentage points, e. g., from 85% to 88% or from 88% to 90%, is of very great technical and economic importance.

Representative present bleaching practice consists in treating a degritted crude clay slip from which an additional coarser particle fraction amounting to about 20% to 30% of the degritted crude clay weight has preliminarily been removed as a substantially unbleachable component, according to prior art, with a reducing agent such as zinc or sodium-hydrosulphite together with an acidic material such as aluminum sulphate or sulphuric acid. By the term hydrosulphite I refer to the salts of hydrosulphurous acid,  $H_2S_2O_4$ . The acid condition established in the slip is maintained at about pH 4. Care is taken to avoid the use of an excess of hydrosulphite and, in general, the practice has been to use 4 to 6 lbs. of  $SO_2$  as hydrosulphite to the ton of clay (weights on the dry basis) when bleaching secondary clays such as Georgia "Fall-line" clays. If larger amounts of hydrosulphite than this are used under these prior art conditions of acidity, etc., on clays such as, for example, sec-

2

ondary Georgia "Fall-line" clays the gray coloration develops. In fact, in order to avoid the formation of gray coloration, it has been preferred practice to use insufficient hydrosulphite even for a complete reducing action if necessary, and thus to avoid the gray coloration and leave a residual buff color which is preferable to the gray for most commercial uses.

I have made the surprising discovery that a clay slip which has been heavily bleached to a pronounced grayness contains two fractions, one of which is markedly gray and of poor color and the other of which is relatively free from gray and poor color and hence of an improved order of brightness, and that these fractions may be separated so as to produce from a given crude clay a product which is markedly superior to that obtainable from the crude by present methods.

I preferably employ hydrosulphite additions within the range which was formerly believed to be incompatible with the production of high quality clay. For secondary clays such as those found along the Georgia "Fall-line," I have used hydrosulphite additions of 10 to 30 lbs. of active  $SO_2$  per ton of dry clay as distinguished from the prior art where additions of 8 lbs. of active  $SO_2$  as hydrosulphite were considered dangerously large.

25 I preferably bleach when the slip is maintained at a pH in the range 2.5-3.2, for a period of at least 10 minutes after bleaching action begins. This acidity may be brought about by the addition of an acid or acidic material; mineral acids such as sulphuric are generally less costly and to be preferred. Although subsequent physical removal of the gray component is not precisely, and in the most minute degree, dependent and contingent upon the use of the larger quantities of hydrosulphite and lower pH than characterizes the prior art, its formation and removal attains technical importance and yields maximum benefits only subsequent to the use of my very drastic bleaching treatment. However, if the pH is not lowered along with increasing amounts of hydrosulphite (in the range previously considered unsuitable), there is no corresponding reduction in the buff color. The virtue of the lower pH, together with the large hydrosulphite additions, appears to be in the greater reduction in buff color which results. To remove the gray component coincidentally formed, I first redisperse the clay after the above overbleaching treatment by adding an alkaline agent such as ammonia or other suitable alkali to readjust the pH of the slip to about pH 5.5 to pH 8.5 (preferably to neutral or slightly alkaline), in the presence of a small amount of dispersing agent such as a few tenths of a per cent of a polyphosphate, sodium hexametaphosphate, etc. Dispersion is, of course, hastened by vigorous mechanical agitation of the mixture. When the clay has been redispersed, a strongly discolored sediment may be separated by allowing the mixture to stand

30 quietly until a gravity separation is effected, or by subjecting the clay slip to a centrifuging action. When the sediment is separated by gravity settling, the supernatant clay is poured off, coagulated, filtered and dried.

35

The dried clay resulting from this treatment is found to have a brightness 3% to 4% higher than the same type of clay as bleached by prior art. This difference in brightness is very important in the paper coating field where brightness is always at a premium.

Another and very material advantage in my invention arises from the fact that, whereas the prior art teaches the separation of the coarser particle size fraction from the crude clay after degritting but before bleaching, my process may be applied to the entire degritted clay including coarse particles. By the prior practice, about 30% of the degritted clay is discarded as coarse particles to which prior bleaching practice was unsuitable, whereas by my process not more than 10% and usually about 5%

or less of the entire weight of the degritted clay is discarded as the discolored fraction, leaving the remaining 80% or more of the clay as well bleached and of good brightness. These yields naturally are somewhat dependent upon the quality of the crude clay.

## EXAMPLE 1

A quantity of crude secondary clay from the Georgia "Fall-line" was mixed with water to make a conveniently handleable slip (about 25% slip in clays of this type). The slip was subjected to a stirring and shearing action in the presence of 0.3% polyphosphate as a dispersing agent. The dispersed clay was then allowed to stand quietly to permit degritting by gravity settling. All of these steps are well known in the prior art.

I next diluted the degritted slip to form a 15% slip and added 0.65% active SO<sub>2</sub> as dry zinc hydrosulphite based on the dry weight of the clay. Sufficient sulphuric acid was added to bring the pH to about pH 2.5 to pH 3.2. The slip was stirred gently to mix the hydrosulphite and acid with the slip and allowed to stand about 30 minutes. At the end of this time the slip was neutralized with ammonia and about 0.5% of polyphosphate added to act as a dispersing agent.

After the dispersion of the slip was effected, it was allowed to settle and a fraction separated by sedimentation. The supernatant suspension was separated from the discolored sediment, coagulated, filtered and dried.

A control slip of the same clay was subjected to the bleaching treatment of the prior art, that is to say, it was degritted, coarse particles removed in an amount of about 30% of the total weight, inasmuch as by prior art this component is considered as relatively unbleachable and is removed prior to bleaching, and the remaining slip brought to a pH of about pH 3 to pH 4 and about 0.25% of active SO<sub>2</sub> as hydrosulphite added. The resulting product was filtered and retained.

The two samples so treated were dried and the brightness was determined by a General Electric Reflection meter using a wave length of about 457 millimicrons with the results shown in Table A.

Table A

|                                    | Brightness, Percent | Discard of Unbleachable Clay, Percent | Bleached Clay Recovery on Degritted Slip, Percent |
|------------------------------------|---------------------|---------------------------------------|---------------------------------------------------|
| Slip treated by my invention       | 87.8                | 2.5                                   | 97.5                                              |
| Slip bleached by prior art process | 83.3                | 30.0                                  | 70.0                                              |
| Difference in brightness           | 4.5                 |                                       |                                                   |

## EXAMPLE 2

I have taken a good quality finished, bleached, and centrifugally fractionated clay which according to prior art was well bleached and separated from coarse particles and upon applying my process to this clay effected a very substantial improvement in brightness after the removal of a considerable amount of discolored matter.

A commercially finished bleached and centrifugally fractionated clay of standard quality which according to prior art was well bleached and separated from coarse particles was treated by my process with a further very substantial improvement in brightness as shown in Table B.

Table B

| Brightness after prior art bleach | Brightness after treatment according to present invention | Brightness Improvement |
|-----------------------------------|-----------------------------------------------------------|------------------------|
| 85.8                              | 88.8                                                      | 3                      |

## EXAMPLE 3

I have also taken a crude secondary clay of quality below that considered standard for bleaching clay according to the prior art, and by applying my process arrived at a bleached clay result well above that produced by prior art processes.

A degritted clay slurry of this quality was treated with 1.0% of active SO<sub>2</sub> as zinc hydrosulphite, and sufficient sulphuric acid to establish an initial pH of 2.8. This pH of 2.8 was maintained by subsequent small additions of sulphuric acid over a period of 15 minutes subsequent to the start of the bleaching reaction. These latter additions of acid were made to restore the condition of acidity as the bleaching reaction tends to reduce the acidity as it progresses. The reaction was then allowed to go to completion by standing without further additions overnight. The bleached clay was neutralized and dispersed and the gray, discolored component removed as previously described. The bleaching results obtained on this clay as compared with bleaching results obtained by the prior art process are illustrated in Table C. Brightness measurements on the removed gray discolored component after filtering and drying gave a brightness of 80%.

Table C

| Brightness after prior art bleach | Brightness after treatment by process of present invention | Brightness Improvement |
|-----------------------------------|------------------------------------------------------------|------------------------|
| 84.0                              | 89.3                                                       | 5.3                    |

Similar improvement in brightness may be achieved on clays which according to the prior art are considered of good quality for bleaching.

## EXAMPLE 4

A ceramic clay of the secondary Georgia type was treated as were the clays of Example 1. Here again the improvement in brightness in the fired ceramic clay was sufficient potentially to put the secondary ceramic in a new technical and market position as indicated in Table D.

Table D

|                                   | Time of Firing, hrs. | Temperature, ° F. | Brightness, Percent |
|-----------------------------------|----------------------|-------------------|---------------------|
| Clay treated by my process        | 2                    | 2,340             | 85                  |
| Clay treated by prior art process | 2                    | 2,340             | 80                  |

In other instances I have found that certain poor colored clays which the prior art treatment is unable to bring to the required level of brightness have been made commercially acceptable in brightness by my treatment.

My researches have shown that the discolored sediment which results from my treatment is not identical with the coarser particles of clay which would ordinarily settle on long standing in clays not treated by my process. I believe that the discrimination depends upon the reaction of the excess hydrosulphite in acid solution of pH 2.5 to 3.2 with the fixed or insolubilizable iron which probably exists in association with other extraneous minerals or even with clay particles as a surface film of hydrous ferric oxide which is known to exist in very stable colloidal suspension. It is probable that several forms of reduced sulphur compounds are produced by the reaction of the hydrosulphites in acid solution and that these substances then react with the iron surfaces to form hydrophobic and hence unstable interfaces in colloidal suspension. It is therefore probable that these iron-bearing particles thereupon agglomerate and fall out

of suspension. Although this theory is consistent with the observed facts, and with the theories of colloidal chemistry, I do not bind myself to this theory.

It will be understood that while I have illustrated and described the presently preferred application of my invention, it may be otherwise embodied or practiced within the scope of the following claims.

I claim:

1. A method of treating clay comprising the steps of forming an aqueous slurry of the clay to be treated, bleaching the slurry with a hydrosulphite bleaching agent until the slurry contains two fractions in suspension one of which is predominately gray in color, all the while maintaining the pH below 3.2, adjusting the pH to the range 5.5 to 8.5 and separating the predominately gray fraction from the slurry by sedimentation. 15

2. A method of treating clay comprising the steps of forming an aqueous slurry of the clay to be treated, adding sufficient zinc hydrosulphite to produce about 1.0% SO<sub>2</sub> adjusting the pH of the slurry to about 2.8 with sulfuric acid, maintaining the pH of the slurry to within the range 2.5 to 3.2 by additions of sulfuric acid while, bleaching the slurry with a hydrosulphite bleaching agent until the slurry contains two fractions in suspension one of which is predominately gray, adjusting the pH to the range 5.5 to 8.5 and separating the gray fraction from the slurry by sedimentation. 20

3. A method of treating clay or the like comprising the steps of forming an aqueous slurry of the clay to be treated, adjusting the pH of the resulting slurry to about pH 2.5 to pH 3.2, adding to the slurry a solution of hydrosulphite whose dry weight content of SO<sub>2</sub> is in excess of 0.4% of the dry weight of the clay to form two fractions in suspension one of which is predominately gray, redispersing the resulting mixture after adjusting its pH to about pH 5.5 to pH 8.5, and separating the resulting gray fraction by sedimentation. 30

4. A method of treating clay or the like to improve its brightness comprising the steps of forming an aqueous slurry of the clay to be treated, adjusting the pH of the resulting slurry to about pH 2.5 to pH 3.2, adding to the slurry a solution of active SO<sub>2</sub> as hydrosulphite whose dry weight content of SO<sub>2</sub> is about 0.4 to 1.5% of the dry weight of the clay to form two fractions in suspension one of which is predominately gray, redispersing the resulting mixture after adjusting its pH to about pH 5.5 to pH 8.5 and separating the resulting gray fraction by sedimentation. 40

5. A method of treating clay or the like to improve its brightness comprising the steps of forming an aqueous slurry of the clay to be treated, adjusting the pH of the resulting slurry to about pH 2.8, adding to the slurry a solution of active SO<sub>2</sub> as hydrosulphite whose dry weight content of SO<sub>2</sub> is about 0.4 to 1.5% of the dry weight of the clay to form two fractions in suspension one of which is predominately gray in color, redispersing the resulting mixture after adjusting its pH to about 55

pH 5.5 to pH 8.5 and separating the resulting gray fraction by sedimentation.

6. A method of treating clay or the like to improve its brightness comprising the steps of forming an aqueous slurry of the clay to be treated, adjusting the pH of the resulting slurry to about pH 2.5 to pH 3.2, adding to the slurry a solution of active SO<sub>2</sub> as zinc hydrosulphite whose dry weight content of SO<sub>2</sub> is about 0.4 to 1.5% of the dry weight of the clay to form two fractions in suspension one of which is predominately gray in color, redispersing resulting mixture after adjusting its pH to about pH 5.5 to pH 8.5 and separating the resulting gray fraction by sedimentation.

7. A method of treating clay or the like to improve its brightness comprising the steps of forming an aqueous slurry of the clay to be treated, adjusting the pH of the resulting slurry to about pH 2.5 to pH 3.2, adding to the slurry a solution of active SO<sub>2</sub> as sodium hydrosulphite whose dry weight content of SO<sub>2</sub> is about 0.4% to 1.5% of the dry weight of the clay to form two fractions in suspension one of which is predominately gray in color, redispersing the resulting mixture after adjusting its pH to about pH 5.5 to pH 8.5, and separating the resulting gray fraction by sedimentation.

8. A method of treating clay or the like to improve its brightness comprising the steps of forming an aqueous slurry of the clay to be treated, adjusting the pH of the resulting slurry to about pH 2.5 to pH 3.2 by the addition of a mineral acid, adding to the slurry a solution of active SO<sub>2</sub> as hydrosulphite whose dry weight content of SO<sub>2</sub> is about 0.4% to 1.5% of the dry weight of the clay to form two fractions in suspension one of which is predominately gray in color, redispersing the resulting mixture after adjusting its pH to about pH 5.5 to pH 8.5, and separating the resulting gray fraction by sedimentation. 35

9. A method of treating clay or the like to improve its brightness comprising the steps of forming an aqueous slurry of the clay to be treated, adjusting the pH of the resulting slurry to about pH 2.5 to pH 3.2 by the addition of a sulphuric acid, adding to the slurry a solution of active SO<sub>2</sub> as hydrosulphite whose dry weight content of SO<sub>2</sub> is about 0.4% to 1.5% of the dry weight of the clay to form two fractions in suspension one of which is predominately gray in color, redispersing the resulting mixture after adjusting its pH to about pH 5.5 to pH 8.5, and separating the resulting gray fraction by sedimentation. 45

| References Cited in the file of this patent |              |               |
|---------------------------------------------|--------------|---------------|
| UNITED STATES PATENTS                       |              |               |
| 2,020,132                                   | Binns        | Nov. 5, 1935  |
| 2,147,774                                   | Lyons        | Feb. 21, 1939 |
| 2,149,506                                   | Bump         | Mar. 7, 1939  |
| 2,251,256                                   | Feldenheimer | July 29, 1941 |
| 2,339,594                                   | Williams     | Jan. 18, 1944 |